

Dec. 15, 1953

D. M. GAGARINE ET AL

2,662,872

MODIFIED METHYLOL MELAMINES AND PROCESS OF MAKING AND USING SAME

Filed Oct. 2, 1950



INVENTORS  
OMITRY M. GAGARINE,  
WILLIAM B. SMITH, JR. &  
MYRTLE J. SPANGLER  
BY

Parrott, Richards & Sims  
ATTORNEYS

## UNITED STATES PATENT OFFICE

2,662,872

MODIFIED METHYLOL MELAMINES AND  
PROCESS OF MAKING AND USING SAME

Dmitry M. Gagarine, William B. Smith, Jr., and  
Myrtle J. Spangler, Danville, Va., assignors to  
Dan River Mills, Incorporated, a corporation  
of Virginia

Application October 2, 1950, Serial No. 187,854

10 Claims. (Cl. 260—67.6)

1

This invention relates to imparting crease-resistance to cellulosic fabrics and more particularly to a water-soluble, thermosetting, synthetic resin which will produce this result on fabrics without lowering the tear strength of the fabric below a permissible minimum.

It has been known heretofore that the crease-resistance of fabrics could be increased practically to any desired extent by treatment of the fabric with a suitable synthetic resin, but the important practical limitation of that process has been the decrease which is simultaneously produced in the tear strength of the fabric as a result of the synthetic resin. For example, in typical prior art processes for imparting crease-resistance to fabrics, the tear strength would be decreased from 50% to 90% and the resulting cloth would be so weak in tear or tensile strength that it would not serve a practical purpose for use in ladies' dress materials, men's shirts and the like.

In accordance with the present invention, the crease-resistance of the cloth may be increased as much as 70% to 100% and the tear strength not decreased more than about 30%. The synthetic resin with which we have been able to obtain these improved results comprises the reaction products of melamine, formaldehyde and urea, and although resins of this general type have been proposed heretofore for treatment of textiles, the above-described long-desired results of high crease-resistance accompanied by high tear-resistance have not been obtained with the prior resins. We have found from extensive research on this problem that the reason for this failure, and likewise the reason for success in the use of the resin of our invention, is the necessity for a very critical control of the amounts or mol ratios of the three constituents.

We found that the desirable end results on the cloth can be obtained only if the above-mentioned three principal resin components are reacted in the mol ratios of 1 mol of melamine to 6 mols of formaldehyde to 3 to 4 mols of urea. It is this critical mol ratio that provides in the final resin the desirable characteristics, and if the amounts are varied substantially from these ratios the desirable high crease-resistance and high tear-resistance of the resin-treated cloth cannot be attained. For example, if more than 6 mols of formaldehyde are used, the tear strength of the fabric will be definitely diminished even though the desired crease-resistance of the fabric is attained. Similarly, but in reverse order, if the amount of urea is reduced

2

substantially below 3 mols, the tear-strength of the cloth will be decreased and, on the other hand, if the amount of urea is increased substantially above 4 mols, the crease-resistance of the cloth will be diminished. Accordingly, to obtain the optimum results characteristic of our invention, the above ratios of 1:6:3 to 4 for the melamine, formaldehyde and urea, respectively, are critical and essential.

10 In preparing the above-described resin of our invention, we have found it advantageous to react the 1 mol of melamine first with the 6 mols of formaldehyde to produce hexamethyol melamine, and then react this intermediate product with the 3 to 4 mols of urea to produce the final resin. In addition to reacting the melamine with formaldehyde to produce the methylol product, we have found it desirable to stabilize that methylolated product by treatment thereof with methyl alcohol or the equivalent to produce dimethyl ether of hexamethyol melamine. Without this ether modification, the finished resin has the objection of being unstable.

15 In preparing the hexamethyol melamine ether condensation product, we may start with straight melamine or with a melamine product which has already been partially methylated and methylolated, for example, the dimethyl ether of trimethylol melamine which is a commercially available product, and treat this with formaldehyde to produce the final hexamethyol product. In any event, sufficient formaldehyde, namely 6 mols, is used to produce the hexamethyol condensation product and without any further methylolation.

20 Illustrative but non-limiting examples for producing the resin products characteristic of our invention are as follows:

## EXAMPLE I

| Constituents                                                | Amount     | Mols | Mol ratio |
|-------------------------------------------------------------|------------|------|-----------|
| Dimethyl ether of trimethylol melamine (80% water solution) | 1,750 lbs. | 5.73 | 1         |
| Formaldehyde (37% water solution)                           | 1,400 lbs. | 17.2 | 3         |
| Urea (dry compound)                                         | 1,035 lbs. | 17.2 | 3         |
| Sodium hydroxide (20% solution)                             | 1,400 mls. |      |           |

25 The dimethyl ether of trimethylol melamine is first reacted with the 3 mols of formaldehyde by mixing and heating the two ingredients, together with the sodium hydroxide which acts as a catalyst, to 157° F. for 15 to 20 minutes. This produces the dimethyl ether of hexamethyol melamine, which is then reacted with the urea by

heating the mixture thereof to 145° F., followed by cooling of the reaction product and storing in drums.

## EXAMPLE II

| Constituents                                                | Amount     | Mols | Mol ratio |
|-------------------------------------------------------------|------------|------|-----------|
| Dimethyl ether of trimethylol melamine (80% water solution) | 1,750 lbs. | 5.73 | 1         |
| Formaldehyde (37% water solution)                           | 1,400 lbs. | 17.2 | 3         |
| Urea (dry compound)                                         | 1,150 lbs. | 19.1 | 3.33      |
| 20% sodium hydroxide                                        | 2,800 mls. |      |           |
| Concentrated hydrochloric acid                              | 1,200 mls. |      |           |

The dimethyl ether of trimethylol melamine is first reacted with the 3 mols of formaldehyde at 157° F. for 15 to 20 minutes, using one-half of the above amount of sodium hydroxide, namely 1400 mls., to produce the intermediate condensation product, hexamethylol melamine. At this point the urea is added with stirring and the temperature kept at 138° F. until all urea has dissolved. Then the hydrochloric acid is added very slowly with stirring, the temperature raised to 155° F., then cooled as rapidly as possible to 80° F. and allowed to stand overnight. The remainder of the 20% sodium hydroxide solution (1400 mls.) is then added, which neutralizes and stabilizes the resinous product.

## EXAMPLE III

| Constituents                      | Amount     | Mols  | Mol ratio |
|-----------------------------------|------------|-------|-----------|
| Melamine                          | 725 lbs.   | 5.73  | 1         |
| Formaldehyde (37% water solution) | 2,800 lbs. | 34.14 | 6         |
| Methyl alcohol                    | 1,800 lbs. | 57.3  | 10        |
| 20% sodium hydroxide              | 1,400 mls. |       |           |
| Concentrated hydrochloric acid    | 600 mls.   |       |           |

In this example, melamine is used as one of the starting materials and is reacted with the 6 mols of formaldehyde to form the hexamethylol product, which is then methylated with the methyl alcohol to produce the methyl ether of hexamethylol melamine. More specifically, the melamine, formaldehyde and sodium hydroxide are heated together to 150° F., until the hexamethylol derivative is formed. The methyl alcohol is then added, and the solution acidified with hydrochloric acid until the pH is between 4 and 5. The solution is then heated until the dimethyl ether is formed and the excess methyl alcohol distilled off. The large excess of methyl alcohol is necessary to insure the reaction taking place.

## EXAMPLE IV

| Constituents                                                | Amount     | Mols | Mol ratio |
|-------------------------------------------------------------|------------|------|-----------|
| Dimethyl ether of trimethylol melamine (80% water solution) | 1,750 lbs. | 5.73 | 1         |
| Formaldehyde (37% water solution)                           | 1,400 lbs. | 17.2 | 3         |
| Dicyandiamide (dry compound)                                | 1,450 lbs. | 17.2 | 3         |
| Sodium hydroxide (20% solution)                             | 1,400 lbs. |      |           |

In this example, dicyandiamide is used in place of urea, but the process is generally the same as that described above in connection with the preceding examples; that is, the dimethyl ether of trimethylol melamine is heated with formaldehyde to 150° F. to form the hexamethylol derivative, and this intermediate condensation product is then reacted with the dicyandiamide by heat-

ing to approximately 170° F. to produce the final reaction product.

The resin prepared in accordance with the above formulas and procedure has definite chemical characteristics which make it suitable for obtaining the desired crease-resistance and tear strength in cloth to which the resin is applied, particularly in terms of the degree of polymerization and the consequent degree of potential reactivity of the resin with the cloth, which may be constructed of any desired type of cellulosic fibers, such as, for example, cotton, rayon and linen. We have found the process of our invention to have substantial commercial value when applied to ladies' dress materials and men's shirting materials made of cotton or viscose rayon or mixtures thereof. The resin is water-soluble and may be applied to any of these cellulosic fabrics in an aqueous solution. The resin is normally substantially neutral, but should be made weakly acid to effect proper reaction with the cellulose of the cloth. For this purpose an acid catalyst such as the amine hydrochloride catalyst manufactured by Monsanto Chemical Company and sold under the trade name "AC" is used. After application of the resin containing this catalyst to the cloth and heating, the catalyst turns the resin slightly acid, which catalyzes the polymerization of the resin and its reaction with the cellulose of the cloth.

Typical crease-resistance and tear strength characteristics of cotton gingham are illustrated by the curves in the accompanying drawing. It can be seen that by using varying amounts of the Resins Nos. I and II, which were produced in accordance with Examples I and II above; the crease-resistance increases from 55% to 93%, while the tear strength decreases from 100% to 40%. The curves show that the greater the amount of resin used, the greater is the crease-resistance, but the lower is the tear strength.

In these curves, complete recovery from creasing (which is never attained in actual practice) is called 100%. Also, the tear strength of the untreated cloth is listed as 100%.

In usual commercial practice it is desirable to have an increase in crease-resistance such as indicated by the use of 10% to 20% of Resin I or II and also not to have the tear strength of the fabric decrease more than the corresponding values for this concentration. More specifically, the two curves for Resins I and II in the accompanying drawing show the following data for crease-resistance and tear strength when the amount of resin used varies from 0 to 40% dry resin based on the weight of the cloth.

## RESIN I

| Concentration, percent dry solids based on weight of cloth. | Tear strength |         | Crease-resistance |
|-------------------------------------------------------------|---------------|---------|-------------------|
|                                                             | Percent       | Percent |                   |
| 100                                                         | 55            |         |                   |
| 90                                                          | 67            |         |                   |
| 80                                                          | 75            |         |                   |
| 70                                                          | 82            |         |                   |
| 67                                                          |               |         |                   |
| 50                                                          | 88            |         |                   |
| 40                                                          | 91            |         |                   |

## RESIN II

|    |    |
|----|----|
| 0  | 55 |
| 6  | 72 |
| 12 | 80 |
| 20 | 87 |
| 30 | 92 |
| 40 | 93 |

5

## THEORY

While we do not wish our invention to be limited to any particular theory, the following discussion of the theory which we conceived agrees with the experimental facts and even with the commercial utilization of the invention.

The resins that have heretofore been used for imparting crease-resistance to fabrics—but which have the objection of decreasing the tear and tensile strength too greatly—include urea formaldehyde, ketone formaldehyde, melamine formaldehyde, other thermosetting formaldehyde condensation products—even formaldehyde itself has been used. These have all been applied to cellulosic fabrics in aqueous solutions and thereafter polymerized to an insoluble state by heating under acid conditions. All of the above-mentioned products have a methylol ( $\text{CH}_2\text{OH}$ ) group and it is believed that the  $-\text{OH}$  radical of the methylol group reacts with an H atom of the hydroxyl group of a cellulose molecule, splitting off water and chemically combining the resin molecule and the cellulose molecule. By having a single resin molecule react with two or more cellulose molecules, the cellulose molecules are cross-linked to form a fairly rigid, three-dimensional net-work. This is illustrated below where a resin molecule



with two methylol groups attached to a resin nucleus R serves to cross-link two cellulose molecules



where OH shows the position of one of the hydroxyl groups in the cellulose molecule and



Cellulose molecules are long and thread-like, so consequently offer little resistance to bending, but offer considerable resistance to pulling apart. This is evident from its mechanical structure.

There are a multiplicity of hydroxyl groups on a cellulose molecule, so it is possible to cross-link several cellulose molecules together with resin molecules to form a fairly rigid, three-dimensional net-work. This cross-linking is illustrated below. The third dimensional cross-linking, that is at right angles to the plane of the paper, cannot be shown, but it is understood that they exist.



6

The very rigidity which gives resistance to bending does not allow the cellulose fibers to distribute the tensile stresses, and materially lowers the tear and tensile strength.

5 If we can maintain this three-dimensional configuration and at the same time make the system more flexible, we will maintain the crease-resistance and regain some of the loss in tear and tensile strength. This can be done by making the  
10 resin cross-linkages between the cellulose molecules longer and more flexible. Compare the illustration below showing this type of cross-linking with the shorter, relatively inflexible cross-linking shown above.



We have discovered that to obtain this flexible resin cross-linkages, it is necessary to have a certain definite ratio of functional groups within the resin molecule. The ratio which we have found to be satisfactory is at least 2 labile hydrogens to 1 methylol (or equivalent) group. The methylol (or equivalent) group is that functional group which reacts with the hydroxyl group of the cellulose molecule. It is, furthermore, the reaction between the labile hydrogens and the methylol (or equivalent) group which causes the polymerization of resin molecules from low molecular weight monomers.

In so far as we know, this ratio of labile hydrogens to methylol (or equivalent) groups has never been known or understood; nor do any of the prior art resins possess this ratio of labile hydrogens to methylol (or equivalent) groups.

By having this ratio of functional groups within the resin molecule, we accomplish the following:

(A) A resin molecule in a low state of polymerization reacts with a cellulose molecule as shown.



60 (B) Because of the large excess of labile hydrogens on adjacent resin molecules, the resin molecules polymerize, growing larger, longer and more flexible, as shown below.



Eventually this resin molecule, dangling from the cellulose molecule, will react with another similarly attached resin molecule, thus cross-linking the two cellulose molecules with a long, flexible resin-linkage as shown below.



Furthermore, it is the reaction between the labile hydrogens and the  $\cdot\text{OH}$  radical of the methylol groups that causes the resin molecules to polymerize into relatively large, water-insoluble molecules.

The above theory may perhaps be better understood by reference to the following illustration of the chemical reaction which is believed to take place when the resin components of Example I above are reacted:



When this intermediate condensation product, that is, the dimethyl ether of hexamethylol melamine, is reacted with 3 mols of urea as described in Example I above, the following type of resinous product results:



It can be seen from the above that the resin has one methylol group and two methylol-methyl ether groups which are the equivalent of methylol groups in that they undergo the same reactions at a slightly higher temperature; six primary amino hydrogens; and three secondary amino hydrogens, all of which are labile. This is then in the ratio of three labile hydrogens to one methylol group.

It must be understood that the above structural formulae are not precise and exact because the resin is slightly polymerized. These structural formulae are, however, indicative of what actually happens and illustrative of our invention.

We claim:

1. A process of producing a water-soluble, thermosetting, synthetic resin forming material suitable for treatment of cellulosic fabrics to provide crease-resistance in the fabric and with limited decrease in the tear strength of the fabric, comprising reacting 1 mol of melamine with 6 mols of formaldehyde to produce hexamethylol melamine and reacting that product with 3 to 4 mols of urea, the reaction with the urea being completed in the presence of an amount of acid sufficient to react all urea with the hexamethylol melamine but insufficient to convert the reaction product to the infusible and insoluble state.

2. A process of producing a water-soluble, thermosetting, synthetic resin forming material suitable for treatment of cellulosic fabrics to provide crease-resistance in the fabric and with limited decrease in the tear strength of the fabric, comprising reacting 1 mol of melamine with 6 mols of formaldehyde to produce hexamethylol melamine, stabilizing said hexamethylol melamine by reacting with methyl alcohol, and then reacting this stabilized hexamethylol melamine with 3 to 4 mols of urea in the presence of an acid under such conditions as will completely react up to 4 mols of urea with said hexamethylol melamine but in an amount insufficient to insublilize the reaction product.

3. A process of increasing the crease-resistance of cellulosic fabrics accompanied by only limited reduction in the tear strength of the fabric, comprising applying to the fabric an acid-reacting catalyst and aqueous solution of a thermosetting synthetic resin forming material composed of the reaction products of 1 mol of a hexamethylol melamine and 3 to 4 mols of urea, heating the cloth treated with this resin forming material to effect polymerization and reaction thereof with the cellulose of the fabric.

4. A cellulosic fabric having relatively high crease-resistance and tear strength, impregnated and reacted with a thermosetting synthetic resin composed of the reaction products of a hexamethylol melamine reacted with from 3 to 4 mols of urea, under such conditions that all free urea is reacted with the melamine.

5. A water-soluble, thermosetting, synthetic resin forming material, consisting of the reaction product of 1 mol of hexamethylol, methylated melamine and 3 to 4 mols of urea, said resin forming material being adapted to be applied to textile fabrics for increasing the crease-resistance thereof while retaining the necessary tear strength of the fabric.

6. A non-free urea containing water-soluble, thermosetting, monomeric, synthetic resin forming material, consisting of the reaction product of 1 mol of dimethyl ether of trimethylol melamine, 3 mols of formaldehyde, and 3 to 4 mols of urea, said resin forming material being adapted to be applied to textile fabrics for increasing the crease-resistance thereof while retaining the necessary tear strength of the fabric.

7. A process of producing a water-soluble, thermosetting, synthetic resin forming material, comprising reacting 1 mol of melamine with 6 mols of formaldehyde and 2 mols of methyl alcohol to produce the dimethyl ether of hexamethylol melamine, and then reacting 1 mol of this dimethyl ether of hexamethylol melamine with 3 to 4 mols of urea under mild acid conditions.

8. A process of producing a water-soluble, thermosetting, synthetic resin forming material, comprising reacting 1 mol of dimethyl ether of trimethylol melamine with 3 mols of formaldehyde to produce the dimethyl ether of hexamethylol melamine, and then reacting 1 mol of said dimethyl ether of hexamethylol melamine with 3 to 4 mols of urea under acid conditions.

9. The process of producing a water soluble heat-setting resin-forming material which comprises reacting 1 mol of a hexamethylol melamine with from about 3 to 4 mols of urea, the reaction conditions being such that all free urea is combined with the hexamethylol melamine.

10. A water soluble reaction product of 1 mol of a hexamethylol melamine and from about 3 to 4 mols of urea, said reaction product being

characterized by the absence of any free urea and by its ability to produce a high degree of crease resistance with a minimum reduction in before strength when applied to cellulosic textile fabrics and polymerized in situ.

DMITRY M. GAGARINE.  
WILLIAM B. SMITH, JR.  
MYRTLE J. SPANGLER.

## References Cited in the file of this patent

## UNITED STATES PATENTS

| Number    | Name      | Date          |
|-----------|-----------|---------------|
| 2,328,424 | D'Alelio  | Aug. 31, 1943 |
| 2,456,568 | Scott     | Dec. 14, 1948 |
| 2,466,457 | Lynn      | Apr. 5, 1949  |
| 2,504,857 | MacIntyre | Apr. 18, 1950 |
| 2,545,450 | Dalton    | Mar. 20, 1951 |

## FOREIGN PATENTS

| Number  | Country       | Date         |
|---------|---------------|--------------|
| 623,361 | Great Britain | May 17, 1949 |